

# UNITED STATES PATENT OFFICE.

GEORGE P. HEMSTREET, OF HASTINGS-UPON-HUDSON, NEW YORK, ASSIGNOR TO THE INTERNATIONAL PAVEMENT COMPANY, OF HARTFORD, CONNECTICUT, A CORPORATION OF CONNECTICUT.

## BITUMINOUS PAVING.

1,000,520

Specification of Letters Patent. Patented Aug. 15, 1911.

No Drawing.

Application filed February 18, 1905. Serial No. 246,333.

To all whom it may concern:

Be it known that I, GEORGE P. HEMSTREET, a citizen of the United States, residing at Hastings-upon-Hudson, in the county of 5 Westchester, State of New York, have invented an Improvement in Bituminous Paving, of which the following description is a specification.

My invention relates to bituminous paving of which the well-known asphaltic pavement, either in sheet or block form, is an example.

Asphaltic pavement compositions, as ordinarily used, comprise a body material, 10 usually crushed stone if the pavement is to be of the block type; and sand, if it is to be of the sheet type, a proper percentage of what are known as fines comprising the fines that may be mixed with and result from the 15 reduction of the stony materials together with any additional amount, usually limestone dust, which may be added to make up the required proportion; with an asphaltic binder or cement to unite the mass into a 20 compact whole. In preparing this paving composition, as, for example, for block or tile purposes, the body material is commonly first heated and placed in a suitable mixer, usually the ordinary pug mill and is dry- 25 mixed. When thoroughly dry-mixed and while under agitation in the pug mill, the asphaltic cement, usually composed of one of the asphalts together with a proper percentage of residuum or other flux, is poured 30 into the agitated mass and the whole thoroughly mixed until the surfaces of all the stony particles both coarse and fine, are completely coated with the cement. The entire 35 mass is now conducted by suitable means to the press, in which it is compressed under 40 heavy pressure into blocks or tiles of the required dimensions. After the compressed blocks or tiles have been cooled, usually in running water, the stony body materials 45 thereof are found usually to be so completely united by the cement that a fracture of a block will cause the fracture of the larger particles of stone, rather than the separation of the stony particles one from another by 50 failure of the cement to hold them. It has been found in practice that the longer the mass remains in its compressed condition, the more completely does the cement become 55 set. In compressing these blocks or tiles, the composition, which reaches the press in

a granular heated condition, frequently varies in consistency, owing to changed conditions of temperature, moisture and the like, and results in a considerable percentage of seconds, or blocks that are more or less 60 imperfect or under or over size. So also the repairs and renewals of pavements once laid result in the collection of a considerable quantity of partially worn blocks, defective 65 because of their reduced size or broken corners, broken in removing or under exceptional traffic but otherwise solid and enduring because the cement has become thoroughly and permanently set. Many attempts and much experiment have been 70 made to utilize these damaged or old blocks, in the making of new blocks, and this experiment and effort has been justified because of the substantial results that would flow therefrom. So far as known to me, 75 however, all these efforts previous to mine have been unsuccessful and for the reason that no practicable way of reducing the blocks to a granular condition has been found. It has been found that the blocks 80 cannot be heated in their full sized condition and thereby reduced for the reason that it takes so long for the heat to penetrate to the interiors of the masses that the exterior portions become too soft and lose many of 85 the lighter oils in volatilization. On the other hand, it has been attempted to crush the blocks in crushing machines down to a degree of fineness substantially the same as when the stony particles were first introduced to the press but here it has been found that the finely crushed masses have presented so many new broken stony faces to be re-coated with cement that the whole amount 90 of cement required in the new blocks would be abnormal and the resultant blocks unduly 95 soft and uncommercial. I have discovered, however, that if the old or previously compressed blocks be broken in a crusher into small pieces, say measuring from one to two 100 inches in diameter, that the amount of broken stony surfaces thereby produced, is not sufficient to require an undue amount of cement in the ultimate mixture, yet when so reduced the masses may be passed through a stone heater and sufficiently and uniformly heated through and through so that when they issue from the heater they are in a granular condition and nearly though not quite as soft and flowable as the new mix- 105

ture but sufficiently so to enable the same to be added in proper proportions to and mixed with the new mixture in the pug mill and the whole thoroughly intermixed and incorporated and afterward pressed as before into blocks or tiles. Of course the proportion of cement first placed in the pug mill somewhat exceeds what would be required if none of the old materials were to be incorporated therewith; this excess being sufficient merely to coat the freshly broken stony surfaces of the old material and at the same time flux the same, so to speak, or soften it to that extent necessary to enable it to be handled properly.

In carrying out this process extensively, as I have, I have been able to use all seconds or old blocks, and thereby economize in the ultimate cost of blocks suited for paving notwithstanding the increased cost of handling the materials which results from the breaking and heating of the old blocks. I have also found what is also of importance, namely, that the blocks in which this old material is incorporated as above described, are superior to blocks otherwise similarly made but wholly of new materials; and this I attribute to the fact that the first compression of the blocks followed by a certain period of set before they are again utilized, gives the binder opportunity more thoroughly and permanently to unite the stony particles in a permanent and enduring manner and that this permanency is not destroyed by the subsequent recrushing and reheating, but softens merely to a sufficient extent to enable it to be remixed with the new material without losing that intimacy and permanency of binding effect which resulted from the first compression and subsequent period of set. When subjected in the new mass to a further compression, this intimacy and permanency or cementitious union is rendered even more complete and the average for the block becomes higher than as if wholly made from new materials.

In carrying out my invention the proportions of the various elements employed may be varied as occasion may require. The following example has shown excellent results: Take 85% more or less of freshly crushed and partly pulverized rock reduced to the usual sizes and mix the same with 4½ to 5% more or less of limestone dust or fines, mixing the whole thoroughly in a pug mill or suitable mixer; add to this from 11 to 12% of asphaltic cement, which may be composed, for example, of the following elements in the following proportions: 100 lbs. of refined Trinidad Lake asphalt and 8 to 12 lbs. of residuum oil or other flux thoroughly mixed and heated; this cement being added to and mixed with the dry-mixed material in the pug mill, and while still in agitation the old materials prepared as

above stated are added to the mass in the proportion say of 1 of the old to 4 of the new. After the whole has been thoroughly mixed together, it is removed in usual manner and compressed into blocks or tiles or other articles for use.

The old materials when reheated as above described, and reduced to a granular condition, are ordinarily not so mobile as the new mixture with which they are to be incorporated and therefore the proportion in which the old can be added to the new, will vary more or less, according to the mobility of the old. For example: this mobility of the old will depend somewhat upon the character of the heating apparatus employed and also upon the sizes to which the old blocks have been first reduced before the heating. Probably the best results are obtainable by reducing the blocks to such sizes as may be readily penetrated by an even degree of heat, while reducing the number of fractures of the stony material to a minimum that is consistent with so doing.

#### Claims:

1. The improvement in bituminous paving for the utilization of previously compressed paving masses in a new mixture or paving composition which consists in reducing the said masses into relatively small pieces approximately one to two inches in diameter or through dimension, heating the pieces so formed, mixing them with a batch of fresh bituminous paving composition comprising stony materials, fines and a cementitious binder, thoroughly mixed and heated, and compressing the resultant mixture for use.

2. The improvement in the manufacture of paving compositions which consists in heating a body material composed of stony materials and fines, dry mixing the same, adding thereto and mixing therewith a cementitious binder, and compressing the mixture into blocks or tiles, cooling the blocks or tiles so formed, permitting said blocks or tiles to set, breaking the same into smaller pieces exceeding the size produced by grinding or pulverizing, said pieces substantially retaining the permanent union of their stony particles and binder, heating said pieces together uniformly throughout, mixing the same with a fresh batch of the said mixed, heated and uncompressed composition and compressing the thoroughly mixed mass for use.

3. The improvement in the manufacture of paving compositions which consists in heating a body composed of stony materials, adding fines including limestone dust, mixing the same, adding a bituminous cementitious binder, and compressing the mixture into blocks or tiles, cooling the blocks or tiles so formed, permitting said blocks or tiles to set, breaking the same into smaller

pieces approximating one or two inches in diameter or through dimension, heating said pieces together uniformly throughout, mixing the same with a fresh batch of the 5 said mixed, heated and uncompressed composition and compressing the thoroughly mixed mass for use.

4. The improvement in the manufacture of paving composition which consists in 10 heating a body composed of stony materials, adding fines including limestone dust, mixing the same, adding a bituminous cementitious binder, and compressing the mixture into blocks or tiles, cooling the blocks or tiles 15 so formed, breaking the same into smaller pieces exceeding the size produced by grinding or pulverizing, said pieces substantially retaining the permanent union of stony particles and binder, heating said pieces together uniformly throughout, mixing the 20 same with a fresh batch of the said mixed, heated and uncompressed composition and compressing the thoroughly mixed mass into bricks or tiles for use.

25 5. The improvement in bituminous paving for the utilization of previously compressed paving masses in a new mixture or composition which consists in reducing the said masses into relatively small pieces, approximately one or two inches in diameter or through dimension, heating the pieces so formed, heating and mixing a batch of freshly crushed and partly pulverized rock, limestone dust and asphaltic cement, agitating said batch, mixing therewith said relatively small pieces of previously compressed paving masses, and compressing the resultant mixture for use.

40 6. The improvement in bituminous paving for the utilization of previously compressed paving masses in a new mixture or composition which consists in reducing the said masses into relatively small pieces, approximately one or two inches in diameter or through dimension, heating the pieces so formed, heating and mixing a batch of freshly crushed and partly pulverized rock, fines and a somewhat excessive quantity of cementitious binder and while the said batch 45 is in agitation, adding thereto said relatively small pieces of previously compressed paving masses and compressing the resultant mixture for use.

7. The improvement in bituminous paving 55 for the utilization of previously compressed paving masses in a new mixture or composition which consists in reducing the said masses into relatively small pieces, approximately one or two inches in diameter or through dimension, heating the pieces so 60 formed, heating and mixing a batch of

freshly crushed and partly pulverized rock, limestone dust and a somewhat excessive quantity of asphaltic cement and, while the said batch is in agitation, adding thereto 65 said relatively small pieces of previously compressed paving masses and compressing the resultant mixture for use.

8. The improvement in bituminous paving 70 for the utilization of previously compressed paving masses in a new mixture or composition which consists in reducing the said masses into relatively small pieces, approximately one or two inches in diameter or through dimension, heating the pieces so 75 formed, heating and dry mixing a batch of freshly crushed and partly pulverized rock and fines, adding to and mixing therewith a somewhat excessive quantity of cementitious binder and, while the said batch is in 80 agitation, adding thereto said relatively small pieces of previously compressed paving masses and compressing the resultant mixture for use.

9. The improvement in bituminous paving 85 for the utilization of previously compressed paving masses in a new mixture or composition which consists in reducing the said masses into relatively small pieces, approximately one or two inches in diameter 90 or through dimension, heating the pieces so formed, heating and dry mixing a batch of freshly crushed and partly pulverized rock and a small proportion of limestone dust, adding to and mixing with said batch a 95 somewhat excessive quantity of cementitious binder, and while the said batch is in agitation adding thereto a less quantity of said relatively small pieces of previously compressed paving masses, and finally compressing the resultant mixture for use.

10. The improvement in the manufacture 100 of bituminous paving which consists in compressing the desired mixture into relatively large masses, such as paving blocks or tiles, permitting them to set in such condition, reducing the same to relatively small pieces or lumps while maintaining the permanent union of the binder and stony particles of the said relatively small pieces or lumps, 110 heating the same, thereby reducing the same to a granular condition, mixing the granular material thus obtained with a fresh and previously uncompressed material and finally compressing the whole for use.

In testimony whereof, I have signed my name to this specification, in the presence of two subscribing witnesses.

GEORGE P. HEMSTREET.

Witnesses:

HARRY STECKERT,  
FRED GORLICH.